

1

3,282,745

**HIGH STRENGTH FABRICATIONS OF ALUMINUM  
BASE ALLOYS CONTAINING COPPER**

George S. Foerster, Midland, Mich., assignor to The Dow Chemical Company, Midland, Mich., a corporation of Delaware

No Drawing. Filed May 27, 1963, Ser. No. 283,595  
9 Claims. (Cl. 148—12.7)

This invention relates to aluminum base alloys and more particularly concerns a novel aluminum base alloy having special utility in the preparation of high strength fabricated articles thereof, and the process for preparing these articles.

Though in general, aluminum base alloys containing copper possess only moderate strength, they are sufficiently strong for certain applications. In other applications requiring higher strength, however, these alloys have heretofore been limited in their utility.

The object of the present invention, therefore, is to provide a novel aluminum base alloy containing copper and capable of being processed to obtain high strength fabrications thereof, and the process for preparing these high strength fabrications.

A novel aluminum base alloy containing copper has now been developed in accordance with the invention wherein the strength has been substantially increased by incorporating therein certain other alloying metals, hereinafter referred to as additive metals, in a specific concentration range which is related to the copper content of the alloy, and processing the so-prepared novel alloy under particular conditions to obtain optimum strength.

All percentages referred to throughout this specification are by weight unless otherwise indicated.

In general, this novel aluminum base alloy contains from at least 4 and preferably at least 5 percent of copper to about 15 percent of copper. The particular amount of copper used depends on the amount and kind of additive metal employed such metal being one selected from the group consisting of calcium, chromium, iron, manganese, mischmetal, nickel, and silicon. The amount of additive metal is generally between 0.3 and 10 percent of the alloy. The balance of the alloy is aluminum.

The minimum amount of copper employed in the alloy is as aforesaid dependent upon the amount of the additive metal if any and is determined in accordance with the empirical equation:

$$\text{Weight percent copper} = 4.0 + KX$$

where X is the weight percent in the alloy of the selected additive metal and K is a constant whose value depends upon the particular additive metal used and the copper content of the alloy, the values for K being hereinafter tabulated as shown in Table I. Preferably, however, the minimum amount of copper to be employed in the alloy is obtained by modifying the above equation by substituting 5 for the 4.

In Table I below, examples of both the operable and preferred concentration ranges for each additive metal, and the corresponding K values therefore are set forth. The 2nd and 3rd columns of proportions are for alloys containing 4% of copper and the 4th and 5th columns are for alloys containing 5% of copper.

2

TABLE I

| Additive Metal  | Operable |           | Preferred |           |
|-----------------|----------|-----------|-----------|-----------|
|                 | Range    | K. Factor | Range     | K. Factor |
| Calcium.....    | 0.4—2.2  | 5.0       | 0.5—1.25  | 8.0       |
| Chromium.....   | 0.3—4.0  | 0.5       | 1.0—3.0   | 1.0       |
| Iron.....       | 1.25—5.0 | 2.0       | 2.0—4.0   | 2.5       |
| Manganese.....  | 1.5—6.0  | 0.5       | 2.0—4.0   | 0.8       |
| Mischmetal..... | 0.5—7.3  | 1.5       | 1.0—5.0   | 2.0       |
| Nickel.....     | 0.5—10.0 | 1.3       | 1.0—6.0   | 1.7       |
| Silicon.....    | 1.5—10.0 | 0         | 2.0—5.0   | 0         |

Depending on the effect desired, other alloying elements conventionally employed can be added to the alloy of the present invention without detracting from its excellent strength properties.

In carrying out the present invention, the novel aluminum base alloy as specified herein is prepared by using the alloying and melting techniques commonly employed in the aluminum art. Highly desirable properties are obtained by rapidly solidifying the molten alloy as, for example, by jet or disc type atomizing devices either in cool air or in a cool inert atmosphere such as, for example, argon. The molten alloy may also be cast into ordinary ingots. However, the strength values thereby obtained are generally less satisfactory than when thin-walled cold molds are used. When the alloy is prepared by atomizing or pelletizing, it is preferred to convert this into massive metal by die expression to obtain maximum properties in fabricated articles, using normal extrusion techniques and equipment. If desired, however, other fabrication methods may be used such as, for example, rolling, forging, or, as above mentioned, casting into thin-walled molds. In the latter method both rapid quenching and fabrication are accomplished in the same operation.

In extruding, the pellets are normally preheated to a temperature within the range of from about 600° F. to about 1000° F., and the extrusion container is at a temperature of from about 500° F. to about 850° F. If desired, the pellets may be precompacted prior to extruding.

In order to obtain optimum strength, regardless of the method of fabrication employed, the alloys of the present invention must thereafter be solution heat treated, rapidly quenched, and aged. Solution heat treating may be accomplished at a temperature within the range of from about 900° F. to about 1000° F. for a period of about one minute or more, followed by rapid quenching and aging the quenched article at a temperature of from about 300° to about 400° F. for a period of from about 5 hours to about 20 hours. Normally the extrude is solution heat treated at about 950° F. for about 15 minutes, water quenched, then artificially aged at 340° F. for 16 hours. However, different heat treatment combinations can be employed, depending on the alloy system being used and the properties desired, without departing from the scope and substance of the invention. If desired, the extrude may be quenched as it emerges from the die then subsequently aged, rather than solution heat treated, quenched, then aged.

The term fabrication as used herein refers to mechanical working procedures such as extruding, casting, rolling, forging, and spinning.

The following examples serve to further illustrate the present invention.

## Example 1

A number of aluminum base alloys containing copper were prepared, each containing a predetermined amount of an additive metal listed in Table I above within the herein specified ranges, and in a proportion relative to that of copper in accordance with the above equation. Each alloy was either cast into ingots (I) 3 inches in diameter or atomized into pellets (P) having a size such that about 85% of the pellets passed through a No. 20 sieve and was retained on a No. 200 sieve (U.S. Standard sieve, fine), while the remainder passed through the No. 200 sieve.

Both the ingots and pellets of the above prepared alloy compositions were extruded by first preheating to about 800° F. then placing the material in the container of a ram extruder, the container being about the same temperature as the pellets, and extruding at a rate of about 5 feet per minute into strip having a rectangular cross section 0.2 inch by 1.0 inch. The resulting strips were then solution heat treated at 950° F. for one hour, quenched, then aged for 16 hours at 340° F.

For comparison both ingots and pellets of the same aluminum base alloy but without any additive metals, were extruded under the same conditions as above, including heat treatment and aging.

Standard test bars of all the alloys prepared as above were made, and tested at room temperature, including the blank or controls aforementioned for comparison, in order to record percent elongation (percent E) (using a 2 inch gauge length), tensile strength (TS), and tensile yield strength (TYS) (at 0.2% offset). Representative results of these tests are presented in Table II which follows:

TABLE II

| Example | Percent Cu | Percent Additive | Form | Percent E | 1,000 p.s.i. <sup>1</sup> |    |
|---------|------------|------------------|------|-----------|---------------------------|----|
|         |            |                  |      |           | TYS                       | TS |
| (Blank) | 5.0        | 2.0 Ca           | I    | 15        | 13                        | 30 |
| (1)     | 12.0       | 1.0 Ca           | I    | 10        | 43                        | 62 |
| (2)     | 12.0       | 1.0 Ca           | P    | 6         | 51                        | 70 |
| (Blank) | 5.0        | 2.0 Cr           | I    | 11        | 27                        | 39 |
| (3)     | 8.0        | 2.0 Cr           | I    | 8         | 40                        | 52 |
| (4)     | 8.0        | 2.0 Cr           | P    | 7         | 55                        | 72 |
| (Blank) | 7.5        | 2.0 Fe           | I    | 16        | 20                        | 42 |
| (5)     | 9.5        | 2.0 Fe           | I    | 10        | 38                        | 56 |
| (6)     | 10.0       | 2.0 Fe           | P    | 8         | 51                        | 70 |
| (Blank) | 4.5        | 3.0 Mn           | P    | 9         | 28                        | 53 |
| (7)     | 7.0        | 3.0 Mn           | I    | 10        | 40                        | 56 |
| (8)     | 8.0        | 3.0 Mn           | P    | 6         | 54                        | 74 |
| (Blank) | 5.0        | 5.0 MM           | I    | 17        | 12                        | 34 |
| (9)     | 10.0       | 3.0 MM           | I    | 12        | 39                        | 60 |
| (Blank) | 5.0        | 3.0 Ni           | I    | 20        | 11                        | 33 |
| (10)    | 10.0       | 3.0 Ni           | I    | 10        | 39                        | 56 |
| (11)    | 15.0       | 3.0 Ni           | P    | 5         | 52                        | 70 |
| (12)    | 5.5        | 5.0 Si           | P    | 10        | 50                        | 69 |

<sup>1</sup> P.s.i.=pounds per square inch of cross section.

It is understood that the copper content in some examples given above may represent an excess of copper with an additive metal over the minimum amount as required in accordance with the above equation.

The figures of the blanks in Table II illustrate the lower strength resulting because of insufficient copper in the alloy. In contrast the alloys of the invention as shown in Examples 1 to 12 inclusive have high strength due to the addition of certain metals when sufficient copper is present as provided for under the present invention, that is, 4 percent or more, or preferably 5 percent or more, but less than 15% of copper.

I claim:

1. A process for preparing high strength aluminum base alloy articles which comprises:

(1) preparing an aluminum base alloy in molten droplet form consisting essentially of from about 4.0 to about 15.0 weight percent copper, from about 0.3 to about 10.0 weight percent of an additive metal, the balance being aluminum, said additive metal

60  
70

5  
4  
being a member selected from the group consisting of calcium, chromium, iron, manganese, mischmetal, nickel, and silicon, the minimum percent of copper being within the range of from about 4.0 to about 15.0 percent and determined in accordance with the equation:

$$\text{Wt. percent copper} = 4 + KX$$

where X is the concentration of the selected additive metal and the corresponding K value for each additive is as follows:

|            |     |
|------------|-----|
| Calcium    | 5.0 |
| Chromium   | 0.5 |
| Iron       | 2.0 |
| Manganese  | 0.5 |
| Mischmetal | 1.5 |
| Nickel     | 1.3 |
| Silicon    | 0   |

20 (2) solidifying the so-prepared aluminum base alloy molten droplets;

(3) and fabricating said alloy into a useful shape by rolling or forging, thereby providing a high strength aluminum base alloy article.

25 2. The process of claim 1 and including the steps of subsequently solution heat treating, rapidly quenching, and aging the fabricated article.

30 3. The process of claim 2 wherein, the solution heat treating is carried out at a temperature within the range of from about 900° F. to about 1000° F. for a period of time of at least about 1 minute, and rapidly quenching the extrude, followed by aging at a temperature within the range of from about 300° F. to about 400° F. for a period of time of from about 5 to about 20 hours.

4. The process of claim 1 wherein, the weight concentration of the selected additive metal in the aluminum base alloy of step (1) is from about 0.4 to about 2.2 percent for calcium, from about 0.3 to about 4.0 percent for chromium, from about 1.25 to about 5.0 percent for iron, from about 1.5 to about 6.0 percent for manganese, from about 0.5 to about 7.3 percent for mischmetal, from about 0.5 to about 10.0 percent for nickel, and from about 1.5 to about 10.0 for silicon.

5. A process for preparing high strength aluminum base alloy pellet extrusions which comprises:

(1) providing in atomized or pelleted form an aluminum base alloy consisting essentially of from about 4.0 to about 15 percent copper, from about 0.3 to about 10 percent of an additive metal, the balance being aluminum, said additive metal being a member selected from the group consisting of calcium, chromium, iron, manganese, mischmetal, nickel, and silicon, the minimum percent of copper being within

the range from about 4.0 to about 15.0 percent and determined in accordance with the equation:

$$\text{Wt. percent copper} = 4 + KX$$

where X is the concentration of the selected additive metal and K for each of said additives is as follows:

|            |     |
|------------|-----|
| Calcium    | 5.0 |
| Chromium   | 0.5 |
| Iron       | 2.0 |
| Manganese  | 0.5 |
| Mischmetal | 1.5 |
| Nickel     | 1.3 |
| Silicon    | 0   |

15

(2) extruding the atomized or pelleted aluminum base alloy thereby to produce a high strength aluminum extrusion.

6. The process of claim 5 wherein, the extrusion temperature is from about 600° F. to about 1000° F.

20

7. The process of claim 5 and including the steps of subsequently solution heat treating, rapidly quenching, and aging the extrusion product.

8. The process of claim 7 wherein the solution heat treating is carried out at a temperature within the range from about 900° F. to about 1000° F. for a period of time of at least about 1 minute, and the extrude quenched,

followed by aging at a temperature within the range from about 300° F. to about 400° F. for a period of time of from about 5 to about 20 hours.

9. The process of claim 6 and including the steps of quenching the extrude, and subsequently aging the so-quenched extrude.

#### References Cited by the Examiner

##### UNITED STATES PATENTS

|           |         |               |           |
|-----------|---------|---------------|-----------|
| 1,480,846 | 1/1924  | Von Zeerleder | 75—139    |
| 1,671,952 | 5/1928  | Brink         | 75—144    |
| 2,062,329 | 12/1936 | Nock          | 75—139 X  |
| 2,249,349 | 7/1941  | Deutsch       | 148—12.7  |
| 2,249,353 | 7/1941  | Fritzlen      | 148—12.7  |
| 2,459,492 | 1/1949  | Bradbury      | 75—139 X  |
| 2,656,270 | 10/1953 | Russell       | 75—139    |
| 2,706,680 | 4/1955  | Criner        | 148—159 X |
| 2,809,891 | 10/1957 | Ennor et al.  | 75—226    |
| 2,865,796 | 12/1958 | Rosenkranz    | 148—12.7  |

##### OTHER REFERENCES

Alcoa Structural Handbook, 1958, page 34.

DAVID L. RECK, *Primary Examiner.*

H. F. SAITO, *Assistant Examiner.*